

## 1

3,703,418

METHOD OF PREVENTING RUST ON  
STEEL SURFACE

Hiroshi Iijima, Masaji Terasawa, Yutaro Gotoh, and  
Osamu Tokita, all % Nippon Kokan Kabushiki Kaisha  
Technical Institute 2730, Kawasaki, Japan  
No Drawing. Continuation-in-part of application Ser. No.  
683,028, Nov. 14, 1967. This application Dec. 31, 1970,  
Ser. No. 103,339

Claims priority, application Japan, Nov. 16, 1966,  
41/74,959

Int. Cl. C23f 7/00

U.S. Cl. 148—6.14

3 Claims

## ABSTRACT OF THE DISCLOSURE

Metals are protected against rust formation thereon by  
immersing them in a molybdate solution.

## RELATED APPLICATION

This application is a continuation-in-part of application  
Ser. No. 683,028, filed Nov. 14, 1967, now abandoned.

## FIELD OF INVENTION

The present invention relates to a process for treating  
surfaces of certain metals to improve the corrosion re-  
sistance thereof by forming a rust-proof film on the metal  
surface by immersing the metals, especially steel and steel  
pipes, in certain molybdate solutions.

## BACKGROUND OF INVENTION

Heretofore, rust-proofing processes have been practiced  
by immersing the metals in a chromate solution to pre-  
vent red rust from forming on cold-rolled steel plates dur-  
ing storage. While most prior rust prevention has been  
effected by chromate treating, metals so treated do not have  
satisfactory adherence with paints when painted there-  
after.

## SUMMARY OF INVENTION

In accordance with the present invention, there is pro-  
vided a process for rust-proofing steel comprising immers-  
ing the steel in an alkaline earth metal molybdate solution.  
The rust-proof film according to this treatment has com-  
paratively good adhesive property with paints. The treat-  
ment is very easily conducted only by immersing a steel  
in a molybdate solution having a definite concentration at  
a definite temperature for an arbitrary time after the steel  
is subjected to degreasing and acid pickling if necessary.  
The concentration of magnesium molybdate solution and  
calcium molybdate solution is preferably within the range  
from 0.025 molar to 0.1 molar and proper temperature is  
within the range from the normal (room) temperature to  
80° C.

It is proved in observation with an electron microscope  
that the film obtained in accordance with the present in-  
vention comprises  $\gamma$ - $Fe_2O_3$ ,  $Fe_3O_4$ ,  $Mo_5O_6(OH)_{10}$ ,  $MoO_3$ .  
The present invention may be applied to plain carbon  
steels, low alloy steels and high alloy steels, etc. Alkali  
molybdate solution is not proper for a molybdate solution  
because the corrosion resistance of a steel treated with  
alkali molybdate solution is not excellent.

The invention is illustrated and in no sense limited by  
the following examples.

## EXAMPLE 1

Cold-drawn steel plate is treated with a molybdate solu-  
tion by immersing it into a solution consisting of  
 $\frac{1}{10}$  molar of magnesium molybdate, calcium molybdate or  
sodium molybdate at 60° C. for such a time as shown in

## 2

Table 1 which shows the results of immersion test and  
wetting test for such reagents.

The tests are conducted under the following conditions:

In the immersion test in running water, the decrease in  
weight ( $mg./cm.^2$ ) resulted from the immersion of  
samples in a water tank having dimensions of 1.0 m. x  
1.0 m. x 0.5 m. (m.=meter) with a flow rate of 125  
cubic centimeter per minute for 10 days.

Wetting test was carried out by leaving samples of the  
plate in a tank maintained at a temperature of 50° C.  
and a humidity of 98% for 24 hours.

Degree of corrosion is shown by the following ratings:

- 15 A—no red rust was produced,  
B—about 2-3% red rust was produced,  
C—red rust was produced all over the surface.

TABLE 1.—CORROSION RESISTANCE WITH MOYBDATE  
SOLUTION TREATMENT

| Reagent                  | Treating period, min. | Immersion test, decrease in weight ( $mg./cm.^2$ ) | Wetting test |
|--------------------------|-----------------------|----------------------------------------------------|--------------|
| Magnesium molybdate      | 2                     | 2.26                                               | B            |
|                          | 5                     | 2.35                                               | A            |
|                          | 8                     | 2.51                                               | A            |
|                          | 10                    | 2.10                                               |              |
|                          | 20                    | 2.28                                               | A            |
|                          | 30                    | 2.56                                               | A            |
| Calcium molybdate        | 2                     | 2.40                                               | B            |
|                          | 5                     | 2.14                                               | B            |
|                          | 8                     | 2.02                                               |              |
|                          | 10                    | 2.01                                               | B            |
|                          | 20                    | 2.54                                               |              |
|                          | 30                    | 2.25                                               | A            |
| Sodium molybdate         | 2                     | 2.75                                               | C            |
|                          | 5                     | 2.66                                               | C            |
|                          | 8                     | 2.88                                               |              |
|                          | 10                    | 2.85                                               | C            |
|                          | 20                    | 2.70                                               | B            |
|                          | 30                    | 2.86                                               | B            |
| Non-treated <sup>1</sup> |                       | <sup>2</sup> 3.04                                  | C            |

<sup>1</sup> Plate used in Example 2.

<sup>2</sup> Hours.

<sup>3</sup> Average for 3 sheets.

45 As shown in Table 1, the effect of treatment varies ac-  
cording to the molybdate solution, and different values are  
shown. In the immersion test, it is proved that corrosion  
resistance is most excellent in a steel treated with alkali  
50 earth molybdate solution, next excellent in a steel treated  
with sodium molybdate solution, and inferior in a non-  
treated steel. Further, the wetting test shows the same  
results. Thus, it is proved that alkali earth molybdate  
solution is proper for a molybdate solution but alkali  
molybdate solution is not proper.

## EXAMPLE 2

Adherence with paint test is conducted on a non-treated  
steel plate, chromate treated steel plate which is com-  
monly marketed, and the present invention steel plate.  
60 Generally, non-treated steel plate has bad corrosion re-  
sistance but is excellent in its adherence with paints.  
Therefore, such a steel is used as a sample in the test  
in order to show excellent adherence with paints. Steels  
subjected to surface treatment generally shows excellent  
corrosion resistance and bad adherence with paints. There-  
fore, chromate treated steel plate is used in the test in  
order to show bad adherence with paints. As steels treated  
65 with alkali molybdate solution show bad corrosion re-  
sistance as shown in Example 1, which is not proper for  
a condition of surface treatment, adherence with paint  
test is not conducted on such a steel. When a non-treated  
steel plate and a steel plate treated with alkali earth

molybdate solution show substantially the same adherence, the latter is regarded as having good adherence.

Sample steel plates are painted with baking type acrylic resin paint and baking type melamine resin paint with an ordinary method and baked. Then, steel plates thus obtained are tested by cross cut test, drawing test and impact test. In cross cut test, a hundred square incisions having an area of 1 mm.<sup>2</sup>, which is deep enough to reach the base plate, are made on the painted surface of the plates to be tested with a diamond needle. Adherence with paints is evaluated by the number of squares left not peeled off.

In drawing test, a diamond needle in contact with the painted surface of the plates to be tested is loaded at the end thereof with a weight of 700 g. placed on a scale, and the needle is rotated in such a way as to describe a circle having a definite diameter on the surface of the plates to be tested which is moved. In such a way, a continuous arc is described on the surface of the plates. Adherence with paints is evaluated based upon the observation of scratches made on the surface of the plates.

Impact test is conducted with an impact tester with 12.5 mm. in diameter of an impact area, load of 300 g. and a height of 500 mm. Elasticity and adherence of paints are evaluated based upon the results of the impact test.

The rating basis of these tests is shown in Table 2.

TABLE 2.—RATING BASIS FOR PAINT ADHERING TEST

| Rating  | Cross cut test | Drawing test                   | Impact test       |
|---------|----------------|--------------------------------|-------------------|
| 10..... | 100            | No abnormal sign.....          | No abnormal sign. |
| 8.....  | 90-99          | Slight peel-off.....           | Swollen.          |
| 6.....  | 80-89          | Peel-off in a small quantity.  | Partial crack.    |
| 4.....  | 50-79          | Peel-off in a medium quantity. | Total crack.      |
| 1.....  | <50            | Total peel-off.....            | Total peel-off.   |

The results of the tests are shown in Table 3.

TABLE 3.—RESULTS OF ADHERENCE WITH PAINTS TEST

[Rating]

| Paint                     | Test                | Kind of steel plate |                     |                              |
|---------------------------|---------------------|---------------------|---------------------|------------------------------|
|                           |                     | Non-treated         | Treated in chromate | Treated in present invention |
| Acrylate resin paint..... | Cross-cut test..... | 8                   | 1                   | 8                            |
|                           | Drawing test.....   | 8                   | 1                   | 8                            |
|                           | Impact test.....    | 6                   | 6                   | 6                            |
| Melamine resin paint..... | Cross-cut test..... | 4                   | 1                   | 6                            |
|                           | Drawing test.....   | 6                   | 1                   | 10                           |
|                           | Impact test.....    | 8                   | 4                   | 8                            |
| Total results.....        |                     | 40                  | 14                  | 48                           |

As shown in Table 3, steel plate treated with chromate shows poor results, while non-treated steel plate shows good results and the present invention steel plate shows the most excellent results. Thus, it is proved that the present invention steel plate is excellent in its adherence with paints.

As may be well understood from the foregoing, steel plate treated with an alkali earth metal molybdate solution has excellent corrosion resistance as shown in Ex-

ample 1 and excellent adherence with paints as shown in Example 2.

As described above, the present method comprises immersing metals, especially steel plates and steel pipes into alkali earth metal molybdate solution, whereupon a rust-proof film such as a molybdenum compound is produced on the surface of the metals. Thus, the corrosion resistance is increased, and rust-proofing is improved. A greater immersion of cold-rolled steel plate into the molybdate solution shows clearly a rust-proof effect. There is no need for high temperature after treatment of the treated steel as with a lithium polymolybdate. The plates or pipes thus treated have excellent adherence with paints, so that this treatment can also be applied as an undercoating for painted metal surfaces.

As indicated by data given above, there is no need for pre-treatment of the steels for corrosion resistance, such as with a solution of a heavy metal salt or with a chromate solution followed by a molybdate solution.

Therefore, the present invention is applicable on an industrial scale.

What we claim is:

1. The process for the provision of a corrosion-resistant film on the surface of steel which consists of immersing the steel, without pre-treatment for corrosion resistance, at a temperature of from room temperature to 80° C. 30 in a solution consisting of an aqueous alkaline earth molybdate solution, wherein the metal is calcium or magnesium, and wherein the concentration of the molybdate solution is from about 0.025 to about 0.1 molar.
- 35 2. The process of claim 1 wherein the molybdate is magnesium molybdate.
3. The process of claim 1 wherein the molybdate is calcium molybdate.

#### References Cited

##### UNITED STATES PATENTS

- |    |           |        |           |            |
|----|-----------|--------|-----------|------------|
| 55 | 2,557,509 | 6/1951 | Miller    | 148—6.24   |
|    | 3,272,663 | 9/1966 | Kronstein | 148—6.16   |
|    | 3,248,249 | 4/1966 | Collins   | 148—6.16 X |
|    | 1,723,067 | 8/1929 | Pacz      | 148—6.14   |

60 RALPH S. KENDALL, Primary Examiner

C. WESTON, Assistant Examiner